

## UNITED STATES PATENT OFFICE

ROBERT WEBER, OF DRENTWEDE, BEZIRK BREMEN, AND FRANZ KINNEBROCK, OF HAMELN, GERMANY; SAID KINNEBROCK ASSIGNOR TO SAID WEBER

## PROCESS FOR THE PRODUCTION OF CLEAN PAPER PULP FROM OLD PRINTED PAPER

No Drawing. Application filed November 13, 1930, Serial No. 495,518, and in Germany November 18, 1929.

Processes are already known in which old printed paper is treated hot or cold with alkali alone or with alkalies with addition of silicates of the series of earth or alkaline 5 earth metals, with or without protective organic colloids. The use of alkaline peroxides together with silicic acid or silicic acid compounds is also known. It has also been proposed to subject old paper first to cooking and 10 then to treat it with Spanish chalk (whiting), or to disintegrate it to fiber in the first stage of the process at a temperature of 80-120° F. and thereafter to treat the paper pulp with a mixture of Spanish chalk and 15 soap.

Finally, it is also known to treat old paper with calcium hydroxide; this latter process, however, has been used only on paper to which the printer's black has been applied by 20 means of a mineral oil. In this connection it is to be remarked that in practice it is not possible to sort the old papers, such as newspapers and the like, according to the kind of adhesive that has been used with the printer's 25 black. This process is therefore applicable only within a restricted range.

Insofar as the known processes contemplate a treatment with use of heat or even in closed container with steam under pressure 30 they involve large extra costs, and in some cases large losses of fibre which in most cases are economically inadmissible. In this connection it is to be noted that the chief item in printed paper is printed newspaper, and that 35 this ordinary paper can furnish only an ordinary, cheap recovery product. Insofar as the purpose is to free the old paper from the printer's black and not to transform the ground wood contained in the paper into cellulose, the ruling principle here is that for 40 economic reasons only the cheapest solvent, the cheapest process, and the most protective treatment of the fibers in order to avoid fiber losses can come into consideration.

Insofar as expensive solvents have to be recovered, it has to be considered that the recovery processes are relatively complicated, that a practically complete recovery of the 45 solvent is impossible, and that the printer's

black and dirt accumulate in the partly recovered solvent means.

It is known that the use of alkali results in a yellowing of the wood fibre; in view of the price of alkali this process therefore involves 55 a large expense, whereas the product has only a small economic value. This yellowing of the fiber is not obviated when organic or inorganic colloids are added to the alkali. Under all circumstances, therefore, the known 60 yellowing of the fiber will occur. The use of these substances will therefore not avoid the above mentioned disadvantages.

It has now been found that these disadvantages can be avoided if the old paper is treated 65 with earth alkali-containing compounds which do not act upon the old paper itself, or if it is treated with only mildly acting solvent means which have a special property for adsorbing printer's black and which 70 have a white coloring power and/or a colloidal character.

The action of these substances on the old paper is a very mild one, so that the wood fibers present in the old paper are not transformed 75 into chemical cellulose. The means are so cheap that it will not be necessary to recover them, and the printer's black is removed in one working operation at ordinary temperature without the fiber being acted on. 80

Such a means, for example, is the causticizing sludge which results from causticizing soda, or the so-called melt from the soda or sulphate process for making pulp cellulose. This sludge is the almost entirely alkali-free 85 residue from the causticization of the soda melt resulting from burning off the waste lye, which, notwithstanding the usual factory practice and the thorough leaching imposed by rational operating principles, still contains 90 some sodium hydroxide, calcium hydroxide and sodium salts, but chiefly lime salts. However, the amount of alkali present is so small that in no case does a yellowing of the fibers take place.

The melts from straw cellulose factories contain silicates on account of the silicic acid contained in the straw. Consequently the causticizing sludge from straw cellulose works 95 also contains silicates principally cal- 100

cium silicates. The colloidal nature of these silicates is very favorable to the removal of the printer's ink. The removal of this latter is, however, also assisted by the presence of suspensions of other lime salts and this because of the power of adhesion and the white coloring properties of these salts.

Magnesium hydroxide has also been found 10 preeminently suitable for the removal of printer's ink from old paper and is very cheap to produce. It may, for example, be obtained from carnallite waste liquors which, after separating out the potassium chloride, 15 contain principally magnesium chloride and which by the addition of alkaline lyes or even causticizing sludge yield the magnesium hydroxide. This has been found to have an especially good coefficient of separation. 20 When making it from carnallite liquor and causticizing sludge there is added to the good separation coefficient another phenomenon which is to be ascribed to the presence of magnesium and lime salts and particularly 25 to the presence of mixtures of magnesium carbonate and magnesium hydroxide. This mixture has quite extraordinary white coloring properties.

The action of causticizing sludge or magnesium hydroxide is further materially increased by adding to these solvents suspensions of such alkaline earth salts as are of a colloidal nature and/or which possess white coloring properties. As salts of a colloidal 35 nature, calcium and magnesium silicates, in particular, may be mentioned and as white color carriers, in particular, barium sulphate, barium carbonate and simple and basic magnesium carbonate. Practical experiments 40 have shown that such suspensions alone (without causticizing sludge or magnesium hydroxide) or when suitably mixed together are capable of loosening and removing the printer's ink. 45 It is obvious that it is also within the scope of this invention to produce the solvents covered by the claims from their components by mixture or by chemical decomposition.

50

*Example*

In a loosening Hollander of the well known type of construction a quantity of old printed paper is softened and disintegrated. During disintegration or after it has been completed 55 the solvent is added and is mixed intimately with the pulp by circulating the pulp in the Hollander. The solvent is, for instance, prepared by mixing about 80 litres of carnallite waste liquor with about 120 litres 60 of causticizing sludge for every 1000 kilograms of old paper. To this mixture are added about 15 kilograms of magnesium carbonate. The concentration of the solvent depends, obviously, on the nature of the paper 65 and of the printed matter to be removed.

After the solvent has been allowed to act for about one hour the paper pulp is washed in the well known way.

The following claims relate to the treating of old paper during and after disintegration. 70

We claim:

1. A process for the production of a pure paper pulp from old printed paper, to which the printer's black has been applied by means of any kind of adhesive, characterized by treating the old printed paper at ordinary temperature in one single operation without any further additions with a dissolving agent which contains practically only alkaline earth compounds with the understanding that in case the hydroxides of the alkaline earth metals are used, the latter have to be of colloidal nature. 75

2. A process for the production of a pure paper pulp from old printed paper, to which the printer's black has been applied by any kind of adhesive, which comprises treating the old printed paper at ordinary temperature in one single operation without any further additions with a dissolving agent which contains practically only alkaline earth compounds selected from a group consisting of colloidal hydroxides of alkaline earth metals, and compounds of alkaline earth 80 metals other than the hydroxides. 85

3. A process for the production of a pure paper pulp from old printed paper, characterized by treating the old printed paper at ordinary temperature in one single operation 90 with a dissolving agent which contains only alkaline earths dissolved colloidal, without the addition of other substances. 100

4. A process for the production of a pure paper pulp from old printed paper, characterized by treating the old printed paper at ordinary temperature in one single operation with a dissolving agent containing only a suspension of alkaline earths possessing 105 white coloring power, without the addition of other substances. 110

5. A process for the production of a pure paper pulp from old printed paper, characterized by treating the old printed paper at ordinary temperature in one single operation 115 with a dissolving agent containing alkaline earths colloidally dissolved, mixed with a suspension of alkaline earths possessing white coloring power. 120

6. For the production of a clean paper pulp from old printed paper a method, wherein the old printed paper is treated with a causticizing sludge obtained as herein described. 125

7. For the production of a clean paper pulp from old printed paper a method, wherein the old printed paper is treated with magnesium hydroxide obtained from carnallite waste liquors and alkaline lyes as herein described. 130

8. For the production of a clean paper pulp from old printed paper a method, wherein the old printed paper is treated with magnesium hydroxide obtained from carnallite waste liquors and causticizing sludge. 70
9. For the production of a clean paper pulp from old printed paper a method, wherein the old printed paper is treated at ordinary temperature in one single operation 10 with a mixture of a suspension containing alkaline earths, and causticizing sludge. 75
10. For the production of a clean paper pulp from old printed paper a method, wherein the old printed paper is treated at ordinary temperature in one single operation 15 with a mixture containing alkaline earths, and magnesium hydroxide obtained from carnallite waste liquors and causticizing sludge. 80
11. For the production of a clean paper pulp from old printed paper a method, wherein the old printed paper is treated at ordinary temperature in one single operation 20 with a mixture of a suspension containing alkaline earths, and magnesium hydroxide obtained from carnallite waste liquors and alkaline lyes. 85
12. For the production of a clean paper pulp from old printed paper a method, 30 wherein the old printed paper is treated at ordinary temperature in one single operation with a mixture of a suspension of colloidal nature containing alkaline earths, and causticizing sludge. 90
13. For the production of a clean paper pulp from old printed paper a method, wherein the old printed paper is treated at ordinary temperature in one single operation 35 with a mixture of alkaline earth silicates and 95 causticizing sludge. 100
14. For the production of a clean paper pulp from old printed paper a method, wherein the printed old paper is treated at ordinary temperature in one single operation 40 with a mixture of an aqueous suspension of calcium silicate and causticizing sludge. 105
15. For the production of a clean paper pulp from old printed paper a method, wherein the old printed paper is treated at 110
- ordinary temperature in one single operation with a mixture of white coloring power containing alkaline earth, and causticizing sludge. 115
16. For the production of a clean paper pulp from old printed paper a method, wherein the old printed paper is treated at ordinary temperature in one single operation 120 with a mixture of a suspension of white coloring power containing alkaline earths, and magnesium hydroxide obtained from carnallite waste liquors and causticizing sludge. 125
17. For the production of a clean paper pulp from old printed paper a method, wherein the old printed paper is treated at ordinary temperature in one single operation 130 with a mixture of a suspension of white coloring power containing alkaline earths, and magnesium hydroxide obtained from carnallite waste liquors and alkaline lyes. 135
18. For the production of a clean paper pulp from old printed paper a method, wherein the old printed paper is treated at ordinary temperature in one single operation 140 with a mixture of alkaline earth carbonates and causticizing sludge. 145
19. For the production of a clean paper pulp from old printed paper a method, wherein the old printed paper is treated at ordinary temperature in one single operation 150 with a mixture of magnesium carbonate and causticizing sludge. 155
20. For the production of clean paper pulp from old printed paper a method, wherein the old printed paper is treated with one or more compounds selected from the group consisting of silicates, carbonates and sulphates of the alkaline earth metals. 160
21. For the production of clean paper pulp from old printed paper, a method 165 wherein the old printed paper is treated with one or more compounds selected from the group consisting of silicates, carbonates and sulphates of the alkaline earth metals mixed with one or more materials selected from the group consisting of causticizing sludge and magnesium hydroxide. 170

ROBERT WEBER.  
FRANZ KINNEBROCK.